

# UNITED STATES PATENT OFFICE.

GEORGE M. MOWBRAY, OF NORTH ADAMS, MASSACHUSETTS.

## METHOD OF PREPARING NITRO-CELLULOSE.

SPECIFICATION forming part of Letters Patent No. 443,105, dated December 23, 1890.

Application filed October 10, 1889. Serial No. 326,609. (No specimens.)

To all whom it may concern:

Be it known that I, GEORGE M. MOWBRAY, a citizen of the United States, residing at North Adams, in the county of Berkshire and State of Massachusetts, have invented new and useful Improvements in the Art, Process, or Method of Manufacturing Nitro-Cellulose or Pyroxyline, of which the following is a specification.

10 The present method of manufacturing pyroxyline on a large scale is to select very fine pure cotton tissue-paper, unsized, of a thickness less than one five-hundredth of an inch, and immerse the same in a bath of sulphuric and nitric acids of certain strength at a given 15 temperature—say about 85° Fahrenheit—for about thirty minutes, to remove from the acid bath, expel the adherent acid, plunge beneath cold water, and wash out all trace of acids by systematic flow of water. Fine pure thin tissue-paper is selected because the instant the paper touches the acid bath it takes on a 20 glutinous or colloid surface, which impedes the thorough conversion of the paper, thin as it is, and thus requires some thirty minutes, or thereabout to enable the conversion to take place through only one five-hundredth of an inch thickness. With thicker paper treated in like manner only the surfaces of a 25 sheet could be nitrated, as the body of the paper would be unacted upon. During immersion the paper has assimilated some forty per cent. of nitric acid, yet at the end of the operation it occupies less bulk than before 30 immersion, so dense and parchment-like has it become. It is this property of the thin film of converted nitro-cellulose protecting the paper beneath from chemical action that has led to selecting so fine a paper and demanded 35 so long immersion, each of these factors adding to the cost of the pyroxyline or gun-cotton.

My invention has for its object the reduction of cost of the crude materials used by substituting a waste product—such as cotton 40 rags, cotton-seed lint from the hulls, &c.—in lieu of high-priced unsized tissue-paper now in use, lessening time now required for conversion, and withal producing a better, because a more uniform, product. These results I attain by availing myself of a phys-

ical effect in crystallizing a salt (preferring nitrates) in the cells of the fiber as a preliminary step to nitration, which opens up these cells to the action of the acid bath, whereby on immersion in the acid bath the sulphuric acid sets free from the salt (if nitrate) nitric acid in a nascent state, which instantly acts chemically on the adjacent walls of each cell wherein the nitrate has crystallized, and thus 55 effect nitration more rapidly, with less costly material, than is possible by the present method of immersing unsized tissue-paper in the usual mixed-acid bath, where the process of nitration is obstructed by the superficial glutinous film of pyroxyline, which forms on 60 the surface of the fibrous sheet of unsized tissue-paper the instant it touches the acid bath.

I do not confine myself to the use of any particular form of cellulose, whether unsized 65 paper, baled cotton, cotton yarn, or textile fabric, as in cotton rags, or even the cotton-lint from cotton-seed hulls obtained by digester process, whether by treatment with sulphurous acid or by caustic soda, or by simple cotton-lint from cotton hulls, as with any 70 one of these forms of cellulose fiber properly cleansed, bleached, and washed, if impregnated with a salt not necessarily, but preferably, a nitrate, a manufacturer can, by adopting 75 my devices, make pyroxyline with less costly cellulose and overcome the inconvenience of that superficial glutinous hinderance to nitration hereinbefore described.

I have said it was not absolutely necessary 80 to use a nitrate. I wish to be understood by this assertion that any salt crystallized, or even water crystallized by freezing in the 85 cells of fibrous cellulose, facilitates nitration by rendering the inner walls of cellular tissue more readily accessible to the acids of the immersion-bath. Some salts it might be necessary to remove after crystallization by washing, while nitrates—sodic nitrate, for instance, for its low price, for its ready crystallization and yield of nitric acid evolved in 90 the acid bath in contact with its sulphuric acid—I prefer to other salts.

To enable others skilled in the art to avail 95 of my invention, I describe it for two varie- 100

ties of pyroxyline—viz., "gun-cotton," and soluble pyroxyline for plastic purposes, respectively.

- For preparing textile cotton for explosive purposes use for one hundred parts of clean dry bleached rags three hundred parts of boiling water and twenty-five to fifty parts sodic nitrate. First dissolve the sodic nitrate in pure clean water, heat to a boiling-point, and gradually introduce the rags, keeping up a moderate circulation of the mass until no more air-bubbles leave the solution. Pass the rags through rollers to remove excess of saline solution. The operator may estimate that rags as they leave the rollers in their wet condition will retain twice their weight of solution. Therefore either by weighing or deducting the proportion of liquid left in the tank he can calculate about the quantity of sodic nitrate taken up by the textile fiber. The rags from the impregnating-tank, having passed through the rollers, are now thrown onto frames protected from dust and allowed to dry gradually, in order to enable the salt to penetrate by the action termed "osmose" into the cells of the fiber and there crystallize. They are then to be thoroughly dried and are ready for the mixed-acids-bath conversion into nitro-cellulose.
- The acids immersion-bath for gun-cotton, (trinitro-cellulose,) as is known in the art, should be as concentrated as possible—say for sulphuric acid, specific gravity 1.84; for nitric acid, specific gravity 1.52, and in the proportion of sulphuric acid two parts, nitric acid one part, both by weight.
- For preparing soluble pyroxyline, (dinitro-cellulose:) use of clean dry bleached rags, one hundred parts; water, three hundred parts; sodic nitrate, from ten to twenty-five parts. The directions given for impregnating, herein-

before described, are to be observed here. The proportions, however, of acids and the strength of the acids immersion-bath differ; for example, sulphuric acid, specific gravity 1.845, sixty-seven parts; nitric acid, specific gravity 1.520, seventeen parts; water, sixteen parts.

It is hardly necessary to remind one skilled in the art that if fine tissue-paper be used, because it is desired to avoid the fine opaque specks found therein by the present process, a weak saline bath, consisting of ten parts of sodic nitrate to one hundred parts of paper, will suffice, and that the drying of the paper should not be too rapid, so as to give time for the osmose action to take place.

Having thus explained my process as I conceive the action to take place and given a full, clear, and explicit description of the mode of proceeding to obtain the advantageous results sought, what I claim in the application, and desire to secure by Letters Patent, is—

In the manufacture of the various grades of nitro-cellulose or pyroxyline, the following process, consisting of three steps: first, a preliminary impregnation of the cellulose material, whether simply fibrous, felted, or textile, by crystallizing a salt, preferably sodic nitrate, in the interstices of the cellulose material; second, immersing this dry saline impregnated cellulose material in a suitable bath of sulphuric and nitric acids, and, third, removing the nitro-cellulose from the saline-acids bath, washing out the adherent acids, and drying the nitro-cellulose, substantially as described, and for the purposes set forth.

In testimony whereof I have affixed my signature in presence of two witnesses.

GEORGE M. MOWBRAY.

Witnesses:

EDWARD BLOSSOM,  
JOHN CARY.